

F. BUTTERWORTH.  
SCREEN FOR CINEMATOGRAPHIC PROJECTION.  
APPLICATION FILED MAY 25, 1915.

1,251,961.

Patented Jan. 1, 1918.



2

Witnesses:  
M. J. Pfeifer.  
H. C. Charles.

Inventor:

Frank Butterworth,  
by Frank S. Anneman,  
atty.

# UNITED STATES PATENT OFFICE.

FRANK BUTTERWORTH, OF LONDON, ENGLAND.

## SCREEN FOR CINEMATOGRAPHIC PROJECTION.

1,251,961.

Specification of Letters Patent.

Patented Jan. 1. 1918.

Application filed May 25, 1915. Serial No. 30,365.

*To all whom it may concern:*

Be it known that I, FRANK BUTTERWORTH, a citizen of United States of America, and resident of London, England, have invented certain new and useful Improvements in Screens for Cinematographic Projection, of which the following is a specification.

This invention relates to improvements in screens for cinematographic projection and has for its object to provide a screen upon which the projected image or picture will be "deeper" than heretofore and the figures in greater relief.

The invention consists broadly in providing a screen with a surface upon which pulverized or granulated glass or other scintillating material is applied or embedded.

In accordance with a practical embodiment of my invention I construct a screen of wood pulp with which granulated or pulverized glass or other such substance is combined. The resulting pulp is rolled into sheets and may be used either alone or may be backed by some suitable fabric or backing. The pulverized or granulated glass is preferably incorporated with the wood pulp throughout a considerable thickness of sur-

face so that the surface of the screen can be cleaned without impairing its utility for the purpose specified.

In the accompanying drawing I have illustrated my invention by a sectional diagram. The numeral 1 designates the front surface upon which the granulated glass is applied or embedded and 2 designates a fabric or other backing. I prefer to employ a fabric backing owing to the facility for rolling thereby afforded, but it will be appreciated that other backings may be employed or the backing can in some cases be dispensed with altogether.

What I claim and desire to secure by Letters Patent is:—

A screen for projecting purposes comprising a front reflector composed of wood pulp and scintillating material intimately mixed and a flexible backing to which the reflector is attached.

In testimony whereof I affix my signature in presence of two witnesses.

FRANK BUTTERWORTH.

Witnesses:

EDWARD A. ELY,  
VINCENT HUGHES.